

[54] **DENSIFICATION OF HARD CHROME PLATED SURFACES**

[75] Inventor: **Louis John Jacobs, Chicago, Ill.**

[73] Assignee: **Combustion Engineering, Inc., Windsor, Conn.**

[22] Filed: **Jan. 2, 1973**

[21] Appl. No.: **320,217**

[52] U.S. Cl. .... **148/6.2, 204/35 R, 204/38 R**

[51] Int. Cl. .... **C23f 7/26**

[58] Field of Search .... **148/6.2; 204/35 R, 38 S, 204/38 R**

[56] **References Cited**

UNITED STATES PATENTS

2,327,885 8/1943 Grace et al. .... 117/71 M X

|           |         |                      |            |
|-----------|---------|----------------------|------------|
| 2,438,013 | 3/1948  | Tanner .....         | 204/35 R X |
| 2,618,578 | 11/1952 | Kreml .....          | 148/6.2 X  |
| 2,746,915 | 5/1956  | Giesker et al. ....  | 204/35 R   |
| 2,755,242 | 7/1956  | Keller et al. ....   | 204/35 R X |
| 2,773,623 | 12/1956 | Schuster et al. .... | 148/6.2 X  |
| 3,526,486 | 9/1970  | Smith et al. ....    | 204/35 R X |
| 3,755,091 | 8/1973  | Austin .....         | 204/35 R X |

Primary Examiner—Ralph S. Kendall

Attorney, Agent, or Firm—Richard H. Berneike

[57] **ABSTRACT**

Porous chrome plated surfaces are densified by treating the surface with a chromic acid solution and heating the part to cure and bring about the conversion of the chromic acid to chromic oxide. The procedure may be repeated as required until the pores and cracks have been filled.

3 Claims, No Drawings

## DENSIFICATION OF HARD CHROME PLATED SURFACES

### BACKGROUND OF THE INVENTION

There are many commercial applications for hard chrome plated parts such as refractory patterns, dies for forming plastic and ceramic parts, hydraulic actuators, cylinder liners, and ball and check valves as well as many other uses. All of the present commercial chrome electroplated surfaces of metal parts contain micropores and a "chicken wire" crazing pattern of cracks which are visible with a low power microscope. It is these inherent defects which cause destruction of the chrome plated surface and failure of the part. Although chromium is very resistant to the corrosive action of many chemicals, such as corrosive acids and alkalies, these chemicals penetrate the pores and cracks and corrode the metal substrate. This action results in the flaking or pealing of the chromium plating from the substrate and parts which are subject to very high pressures, such as hydraulic components, may leak after a short service period.

### SUMMARY OF THE INVENTION

The object of the present invention is to treat chrome plated surfaces to densify the surface by filling in inherent defects such as micropores and cracks. This densification will prevent penetration of the chrome plating by chemicals and thereby reduce the tendency of the chrome plating to become detached from the substrate and reduce chemical attack on the substrate. The objects of the present invention are accomplished by treating the chrome plated surfaces with a chromic acid solution and then converting the chromic acid to chromic oxide.

### DESCRIPTION OF THE PREFERRED EMBODIMENT

The chromic acid solution for use in the present invention is prepared by dissolving chromium trioxide in water to produce a chromic acid solution having a specific gravity of 1.64-1.66 at 70°F. The preferred specific gravity is 1.65. The chrome plated metal part to be treated is then immersed into the chromic acid solution or otherwise treated with the solution and the chromic acid wets and penetrates the micropores and cracks of the chrome plated surface. The treated metal part is then heated so as to convert the chromic acid to a refractory chromic oxide. The conversion of the chromic acid to chromic oxide takes place at a temperature between 700°F and 1,200°F. However, a preferred heating cycle should be followed to obtain the most effective densification. This heating cycle involves first heating the treated metal part to 230°F ± 10°F and held at this temperature for a period of time sufficient to insure that all the moisture is removed from the micropores and cracks of the chrome plated surface. The part is then gradually brought to a temperature of 700°F ± 50°F. The rate of heating to this temperature level is determined by the mass and complexity of the metal part and is selected to avoid thermal stresses. Sufficient time is allowed to stabilize the temperature throughout the metal substrate. After the temperature has stabilized at 700°F ± 50°F, the tempera-

ture of the surface is rapidly brought to 1200°F ± 50°F and then the part is removed from the heating equipment. This rapid heating from 700° to 1,200°F converts the chromic acid to chromic oxide and the chromic oxide becomes very dense and is more strongly bonded to the base metal.

The repeated coating with chromic acid and curing to form chromic oxide will tend to more completely fill the pores and cracks of the chrome electroplated surface. After the first coating has been applied and cured, the part is then cooled to 150°F and again treated with chromic acid solution, heated to 230°F, gradually brought to the stabilized temperature of 700°F and then rapidly heated to 1,200°F. This procedure is repeated until the pores and cracks have been filled. The part may then be finished by polishing by conventional means.

Heating of the metal parts may be accomplished by any conventional means such as in ovens or furnaces, or by means of radiant heat burners or by direct flame. However, parts which have been heated with induction heating have proved to be the most effective in bonding the chromic oxide to the substrate. This fact is apparent on a microscopic examination of sections of parts treated in accordance with the present invention.

It has been found to be helpful in the practice of the present invention to add about 0.05 to 0.5 percent by weight of carbon black or lamp black based on the weight of the chromic acid used to make the chromic acid solution. The presence of the carbon reduces the oxygen content of the solution and in some manner increases the rate of filling of the pores and cracks with chromic oxide.

Although the present invention has been described with reference to specific examples it will be understood that these are merely illustrative and that changes may be made without departing from the invention as claimed.

What is claimed is:

1. A method of treating metal parts having chrome plating thereon wherein said chrome plating contains pores and cracks comprising the steps of:
  - a. applying a solution to said chrome plated metal parts whereby solution penetrates said pores and cracks, said solution consisting essentially of a chromic acid solution having a specific gravity of from 1.64 to 1.66; and
  - b. heating said chrome plated metal parts having said chromic acid applied thereto to a temperature of about 230°F ± 10°F, gradually heating to a temperature of 700°F ± 50°F, permitting said temperature to stabilize at 700°F ± 50°F throughout said part and then rapidly heating said part to 1,200°F to convert said chromic acid to chromic oxide.
2. A method as recited in claim 1 wherein said step of heating comprises the step of heating by induction heating.
3. A method as recited in claim 1 wherein said chromic acid solution contains a material selected from the group consisting of carbon black and lamp black, said material being present in an amount equivalent to 0.05 to 0.5 percent by weight of the chromic acid present in the chromic acid solution.

\* \* \* \* \*